

# United States Patent

Bereczky et al.

[15] 3,637,475

[45] Jan. 25, 1972

[54] ZINC-PLATING BATH FOR BRIGHT OR GLOSSY COATING

[72] Inventors: Tiberiu Bereczky; Ernest Grünwald, both of Cluj; Ioan Crisan, Bucharest, all of Romania

[73] Assignee: Ministerul Industriel Constructiilor de Masini, Bucharest, Romania

[22] Filed: Sept. 25, 1968

[21] Appl. No.: 762,642

[52] U.S. Cl. .... 204/55 R

[51] Int. Cl. .... C23b 5/10, C23b 5/46

[58] Field of Search: 204/55, 43, 44, 114, 116; 106/1

[56]

## References Cited

### UNITED STATES PATENTS

|           |         |                      |          |
|-----------|---------|----------------------|----------|
| 1,380,142 | 5/1921  | Hanson et al. ....   | 204/55   |
| 1,607,869 | 11/1926 | Colcord.....         | 204/55   |
| 1,856,261 | 5/1932  | Phillips et al. .... | 204/55 X |
| 2,871,171 | 1/1959  | Atkinson.....        | 204/52 X |
| 3,296,104 | 1/1967  | Eppensteiner.....    | 204/55   |
| 3,317,412 | 5/1967  | Dahlmann .....       | 204/55   |

Primary Examiner—G. L. Kaplan  
Attorney—Karl F. Ross

[57]

## ABSTRACT

An alkaline cyanide-free zinc electroplating bath. The bath contains sodium hexametaphosphate and such gloss-controlling additives as gelatine, furfural and sulphite liquor from cellulose production.

2 Claims, No Drawings

## ZINC-PLATING BATH FOR BRIGHT OR GLOSSY COATING

### FIELD OF THE INVENTION

Our present invention relates to alkaline zinc-plating baths omitting cyanide for producing bright glossy coatings and, more particularly, to a coating bath and to a method of plating zinc using this bath.

### BACKGROUND OF THE INVENTION

It is known from the literature that the zinc coating of metal parts by acid plating baths with a small dispersion power but high-current density and efficiencies up to approximately 100 percent, produces rough coatings of large crystals which will not always stick. They do not have, for example, the glossy and bright aspect and smooth texture frequently desired.

It has also been proposed to substitute alkaline baths complexed with cyanide ions, in order to form smooth and glossy surfaces. Besides the zinc ions and the cyanide ions such baths contain hydroxyl ions. Such baths may also contain additives influencing the various parameters of the coatings, generally organic and inorganic compounds, capable of modifying the grain size of the deposited zinc or of promoting a glossy coating. Such additives may include aliphatic aldehydes, aromatic aldehydes or ketones, heterocyclic compounds with oxygen, condensed substances with benzene rings, thioureas, the reaction products of heterocyclic aldehydes with nitrogen or aromatic amines or gelatine. Metallic additives include manganese and molybdenum directly or in the form of compounds thereof.

In aqueous baths, the additives are not readily soluble and do not directly determine a glossy finish on the coating. In fact, the coating has a brownish or slightly yellowish coloration which must be removed substantially by treatment of the coating with an inoxidizing agent.

Cyanide-containing alkaline baths also have the disadvantage that they are toxic and cannot be disposed of without difficulty, that they are dangerous to work with, that they have a poor current efficiency, and operate with low-current density. To avoid these disadvantages, it has been suggested to provide alkaline zinc-coating baths without cyanide and using other complexing agents. Zincate baths may operate at efficiencies close to 100 percent, but produce large-crystal dark and spongy coatings. Pyrophosphate baths require such careful control of the plating parameters that they have been found to be impractical. Moreover, admixture with other ingredients is necessary to obtain glossy deposits. The use of aliphatic amines gives glossy zinc coatings at low-current densities, but without a desirably large dispersion power so that with increased current densities brittle coatings are obtained. Much may also be made of the use of sodium dodecyldiphenyloxidizedisulphonate. These baths also have limited value because of the low-current density under which they operate.

### OBJECTS OF THE INVENTION

The principal object of our present invention is to provide an alkaline zinc-plating bath for the production of bright glossy zinc coatings which will obviate the disadvantages mentioned earlier.

It is also an object of this invention to provide a method of plating zinc onto a substrate using an alkaline plating bath which is free from cyanide and yet provides good dispersion power and is capable of the efficient deposition of bright zinc coatings of good mechanical properties at high rates.

### SUMMARY OF THE INVENTION

We have now discovered that these objects can be obtained with an alkaline zinc-plating bath which contains sodium zincate, omits cyanide and utilizes as the complexing agent sodium hexametaphosphate. Surprisingly, the complexing agents tie up the zinc ions as complexes with weak disassociations and thereby reduce the concentration of uncomplexed zinc in

solution. As a result, the cathodic polarization increases and zinc with a fine microstructure structure is deposited.

Advantageously, auxiliary gloss-promoting additives are employed in conjunction with the sodium hexametaphosphate. Typical among these additives are furfural, gelatine and waste sulphitic lye as resulting from the processing of cellulose and utilized in concentrations of 1.0 to 5.0 g./liter. These additives may be used individually or together and, depending upon their relative proportions, produce a gloss ranging in texture from a semigloss to a bright reflective optical gloss. The gloss is formed without subsequent treatment.

More specifically, the alkaline zinc-plating bath according to the present invention contains 40 to 75 g./liter of sodium hydroxide, 10 to 25 g./liter zinc oxide, 30 to 45 g./liter sodium hexametaphosphate and the above-mentioned gloss-promoting additives. It may be noted, incidentally, that other compounds hitherto utilized for promoting gloss may be introduced in place of the three preferred additives mentioned earlier, or together with them. Such compounds include the organic members mentioned earlier and inorganic compounds such as ammonium molybdate and sodium sulfite.

We may also introduce additives for increasing the power of dispersion, the adhesion of the deposit to the substrate and the conductivity of the electrolyte in addition to additives for the prevention of pore formation and wetting agents. The bath may be prepared by combining zinc sulfate and sodium hydroxide, thereupon recovering the zinc-hydroxide. The alkaline zincate solution is mixed with the sodium hexametaphosphate solution whereupon the gelatine solution and furfural solution are added; the sulphitic lye, neutralized with sodium hydroxide is added as the last component. The term "sulphitic lye" as used herein, is intended to refer to the sulphite liquor obtained in the production of cellulose, any acidic character being removed by the neutralization. The bath can be utilized immediately and need not be exposed to electrochemical processing or aging. In use, any losses of the above ingredients from the bath can be made up by corresponding addition of ingredients thereto and we prefer to continuously or periodically filter and recycle the electrolyte during plating.

According to another feature of this invention, the plating temperature is held between 20° and 24° C. so that no heating of the bath is necessary. The cathodic current density is 1 to 4.5 A./dm.<sup>2</sup> where no agitation is provided, but up to 6 A./dm.<sup>2</sup> where drum or other rotative agents are used. For stationary baths, the working voltage is 0.6 to 1.2 volts whereas with agitation it is 6 to 8 volts. Best results are obtained when the plating is carried out to deposit 15 to 60 microns/hour of a coating. The glossier the coating desired, the lower should be the deposition rate. The current efficiency is about 85 percent and the dispersive power is about 40 percent. The coatings have satisfactory uniformity, form well even in interior or hollow portions of the substrate and upon surfaces with high complexity and have good ductility and adhesion. The coating may have a brightness ranging from that of a plated chromium to a semigloss and may be applied to polished or nonpolished surfaces. Suitable substrates are iron, steel and nonferrous metals and alloys, such as copper, aluminum and brass. The coatings can be obtained in various hues, e.g., whitish, yellowish and bluish, and can be substituted in many cases for more expensive cadmium coatings.

The corrosion resistance of the coating and the retention of the gloss may be improved by treatment of the surfaces with oxidizing compounds such as chromic acid and the nitrogen acids, thereby providing a passivating treatment which may be termed chromation or oxidation. The corrosion-resistance of the coating is superior to that obtained with cyanide baths and the plating may be carried out with conventional plating equipment.

## SPECIFIC EXAMPLE

Automotive-vehicle spark plugs, turned from bars of nonalloyed steel on automatic lathes, are coated with zinc in an aqueous bath of the following composition:

15 g./liter technical zinc oxide  
 65 g./liter technical solid sodium hydroxide  
 40 g./liter sodiumhexametaphosphate, 68%  $P_2O_5$   
 4 cc./liter technical furfural  
 4 g./liter food-gelatine sheets  
 2 cc./liter sulphitic liquor obtained from a cellulose production plant, neutralized with 25 percent sodium hydroxide.

To produce 1 liter of the electrolyte, we dissolve, in 300 to 400 cc. of water, the sodium hydroxide and then introduce into this solution the zinc oxide with stirring and agitation. In another 300 to 400 cc. of hot water is dissolved the sodium hexametaphosphate and the two solutions are then combined. The furfural dissolved in about 50 cc. of water and the gelatine dissolved in 50 to 60 cc. of water are added successively to the basic solution to which is thereafter added the sulfite liquor.

Zinc plating is carried out on the article with a current density of 3 A./dm.<sup>2</sup> and a voltage of 1.2 volts with the parts suspended from the cathode bar at a distance of 300 mm. from the anode. The cathode bar is given a reciprocal motion at a frequency of 1 Hz., and an amplitude of 25 mm. The parts were previously subjected to alkaline electrolytic degreasing and slight pickling with hydrochloric acid. Coating was carried out for 10 to 30 minutes whereupon the zinc-coated parts

were removed and washed with cold water. The zinc-coating has a bright color similar to that of glossy chromium, is ductile, adherent to the basic metal and has an effective gloss while the uniformity of the deposit is satisfactory. If lesser quantities of the gloss-promoting additives are used, the coating is a semigloss.

The zinc coating can be passivated by chromation in a bath containing 1.5 g./liter sodium-dichromate, 50 g./liter sodium sulphate, 6 g./liter sodium chloride and 4 cc./liter concentrated sulphuric acid. The treatment was carried out at 20° C. for 12 seconds and a golden hue was imparted to the coating.

We claim:

1. An alkaline cyanide-free aqueous zinc-electroplating bath containing in addition to zincate ions in an amount equivalent to 10 to 25 grams/liter of zinc oxide, 30 to 45 g./liter of sodium hexametaphosphate and a gloss-controlling additive consisting of about 4 grams/liter of gelatine and about 4 cc./liter of furfural.
  2. The bath defined in claim 1 which consists essentially of:
- 15 g./liter zinc oxide,  
 65 g./liter sodium hydroxide  
 40 g./liter sodium hexametaphosphate (68%  $P_2O_5$ )  
 4 cc./liter furfural  
 4 g./liter gelatine and  
 2 cc./liter cellulose-production sulphite liquor neutralized with sodium hydroxide.

\* \* \* \* \*

30

35

40

45

50

55

60

65

70

75